

## UNITED STATES PATENT OFFICE

2,681,895

TRANSPARENTIZING COMPOSITIONS AND  
PROCESS

Robert R. Parmentier, Upper Darby, Pa.

No Drawing. Application January 2, 1952,  
Serial No. 264,659

3 Claims. (Cl. 260—33.6)

1

This invention relates to compositions and processes for transparentizing and sealing fibrous materials such as paper.

It is often desired to reproduce copies of drawings, printed pages, or other similar materials. This may be accomplished by photographing the drawing and preparing prints from the so-obtained negative. A further method is to prepare prints directly from such page or drawing. In this latter method, the paper in general use is too opaque to permit the preparation of satisfactory prints, and in the photographic process the cost of the reproduction makes the process prohibitive in many instances. In order to overcome these and other difficulties, it has heretofore been suggested to employ various compositions in order to transparentize the paper from which reproductions are desired, and thus render the attainment of prints directly therefrom feasible. Compositions heretofore proposed, however, have serious disadvantages which greatly restrict or prevent their use. For example, compositions heretofore proposed suffer one or more of the following difficulties: the compositions may be dangerous to compound and use; are difficult to prepare and apply to the paper; drying thereof is slow; the material used in transparentizing, usually an oil, seeps, i. e., is transferred to prints and other papers which it contacts thus restricting its use and making storage of the treated paper difficult; odor is imparted to the treated paper which makes its use obnoxious and which permeates other papers and materials such as when stored together; the treated paper sticks, i. e. the treated paper sticks to hot surfaces of reproducing machines, which prevents or greatly limits their use in most processes; and the treated paper is not sufficiently transparentized, or is unevenly transparentized, so that suitable reproductions cannot be prepared therefrom.

In patent application, Serial No. 155,565, filed April 12, 1950, now Patent Number 2,616,815 a transparentizing solution comprising mineral oil, 10-35 vol. per cent; toluene, 4-10 vol. per cent; and carbon tetrachloride, 55-80 vol. per cent is described. As further described in said patent application, and as claimed in patent applications, Serial Numbers 190,882 and 190,883, filed October 18, 1950, now Patent Numbers 2,646,363 and 2,646,369 respectively, it is preferred to apply a sealing composition, comprising wax, 2-6 vol. per cent; a gasoline hydrocarbon fraction, 31-47 vol. per cent; and carbon tetrachloride, 47-67 vol. per cent; to paper transparentized by the aforementioned transparentizing solution to prevent seepage.

2

An object of the present invention is to provide compositions effective to transparentize and seal paper which obviates the difficulties encountered with heretofore known compositions. A further object is to provide compositions effective to transparentize and seal paper with a single application. Another object is to provide a process for simultaneously transparentizing and sealing paper.

The novel composition of the present invention comprises mineral oil, 10-35 vol. per cent; benzene, toluene or xylene, 4-10 vol. per cent; carbon tetrachloride, 55-80 vol. per cent; and a small soluble quantity of synthetic rubber. This composition is applied directly to the paper to be transparentized, preferably to the side thereof which does not contain the printed matter or drawing, the reproduction of which is desired. Application is conveniently accomplished by rubbing the paper with a cloth or sponge saturated with the transparentizing and sealing solution. Other means of application may be employed, such as spraying, brushing, and dipping. The composition of the present invention dries in a very short time, within about 1-5 minutes, and the so-treated paper may then be used in preparing photographic reproductions.

An advantage of the composition of the present invention is that the paper is transparentized and sealed by application thereto of a single solution, i. e., the application of a separate sealing composition is unnecessary.

The oil employed in the present composition is preferably a refined white mineral oil boiling in the lubricating oil range. The aromatic component may be benzene, toluene or xylene, usually as a mixture of xylenes, or a mixture of two or all three of the named aromatic hydrocarbons.

The synthetic rubber to employ must be soluble in the liquid components to the extent of at least 0.075 gram per 100 cc. of solution. Polymers of chloroprene, copolymers of butadiene and styrene, and copolymers of chloroprene and isoprene are examples of synthetic rubbers which give good results. Natural rubber and polyvinyl chloride are not sufficiently soluble in the liquid components of the composition to warrant their use.

It is important that the stated concentration ranges for the ingredients of the present compositions be observed. If mineral oil be employed in less than the stated amount, the paper is not sufficiently transparentized to permit satisfactory reproduction, whereas if more than the stated quantity is employed, the paper will be slow drying and seepage occurs; if less than the

stated amount of aromatic, such as toluene, is employed seepage is observed, whereas if more than the stated quantity is employed the composition may be inflammable and have an offensive odor; if carbon tetrachloride is employed in less than the stated quantity, penetration of the paper by the transparentizing composition is decreased thereby making the application of the composition difficult, and the composition may be inflammable, whereas employing more than the stated quantity results in too fast drying which makes its application to paper difficult and uneven. The synthetic rubber should be soluble in the admixture of other components to the extent of 0.075 gram/100 cc., and the operable range is from 0.075 to 1 gram/100 cc., but it will seldom be necessary to dissolve more than 0.3 gram/100 cc. Using concentrations of synthetic rubber lower than the minimum stated, a good seal sufficient to prevent seepage of oil is not obtained, whereas at concentrations above the stated maximum, tacking is observed, and in some instances the synthetic rubber may be removed from the paper surface by rubbing.

In the event that anti-oxidants or other foreign materials have been added to the synthetic rubber, the solution may exhibit a slight haze or cloud. In general, such haze or cloud does not deleteriously affect the present process, but where using relatively high concentrations of synthetic rubber the haze may be objectionable. In such case, the haze may be removed by filtration.

Various papers may be treated in accordance with the present process, and the so-treated papers used in various reproduction processes. Papers which may be treated, for example, include the usual bond paper of say about 13 to 24 lb. weight per 1000 sheets, photographic, tracing, chart and blue print papers, and in general any paper except very heavy fibrous materials such as cardboard. The treated papers may be employed for making reproductions in a variety of processes involving the transmission of light through the treated paper. As illustrative of such processes may be mentioned direct printing such as contact box printing, the use of Ozalid, Bruning, blue print machines and actinic light contact printing. The treated papers may also be used in projection printing.

#### Example I

A series of compositions in accordance with the present invention was prepared and tested. Preparation was by dissolving synthetic rubber in a solution of mineral oil, 28.5 vol. percent; carbon tetrachloride, 66.5 vol. percent; and benzene, 5 vol. percent. Synthetic rubbers used included three different polymers of chloroprene, a copolymer of chloroprene and isoprene, and two different copolymers of butadiene and styrene. Each synthetic rubber was dissolved in concentrations of 0.075, 0.15, 0.30 and 5.0 grams/100 cc. of solution; some compositions were prepared at 0.5 and 1.0 gram/100 cc. concentration.

Photolith copies of engineering drawings on opaque paper unsuitable for direct reproduction were transparentized and simultaneously sealed with the above composition by rubbing the photolith back with a cloth saturated with the composition being tested. Prints were prepared from the transparentized and sealed drawings using a direct printing (Ozalid) machine. It was found that the synthetic rubbers were not sufficiently soluble at 5 grams/100 cc. to pre-

pare suitable solutions; the compositions were colored, viscous, and could not be satisfactorily applied to paper.

At concentrations of 1 gram/100 cc., such as when using a copolymer of chloroprene, good transparency and sealing was observed, but the compositions were relatively difficult to apply, were slightly tacky in some instances, and were not quite as translucent to light as the remaining compositions. Accordingly, use of compositions containing less than 1 gram/100 cc. solution is required.

At concentrations of 0.075, 0.15 and 0.30 gram/100 cc. excellent results were achieved in all instances. The compositions were easy to apply and transparency was obtained. On storage in contact with other paper no seepage from the transparentized and sealed drawings was observed. Prints were prepared from transparentized and sealed drawings at each of the stated concentrations of synthetic rubber and excellent results obtained. None of the transparentized papers exhibited a detectable odor. However, at concentrations of synthetic rubber below the 0.075 gram/100 cc. solution, a slight amount of seepage is observed. Accordingly, use of compositions containing at least 0.075 gram of synthetic rubber/100 cc. of solution is required.

#### Example II

Another series of compositions was prepared identical to the compositions of Example I except that toluene was substituted for benzene. Three separate polymers of chloroprene were employed at concentrations of 0.075, 0.15, 0.30 and 1 gram/100 cc. of solution.

Results substantially identical to those of Example I were obtained.

In both of the above examples, the paper treated was transparentized and sealed to substantially the same extent as when using both the transparentizing composition and sealing composition of aforementioned patent applications, Serial Numbers 155,565, 190,882 and 190,883.

Within the operable ranges of synthetic rubber concentration, the compositions dry practically immediately on application to paper, so that printing may be begun within 1 to 5 minutes after application.

Natural rubber is not soluble in the present solution to the extent of 0.075 gram/100 cc., and hence is not operable. Copolymers prepared from admixtures containing substantial quantities of acrylonitrile and polymers of vinyl chloride likewise are not sufficiently soluble to warrant their use in the compositions of the present invention.

I claim:

1. A transparentizing and sealing solution consisting of from 10-35 vol. per cent mineral oil, from 55-80 vol. per cent carbon tetrachloride, from 4-10 vol. per cent benzene, and from 0.075 to 1 gram per 100 cc. of solution of a synthetic rubber selected from the group consisting of polymers of chloroprene, copolymers of butadiene and styrene, and copolymers of chloroprene and isoprene.
2. A transparentizing and sealing solution consisting of from 10-35 vol. per cent mineral oil, from 55-80 vol. per cent carbon tetrachloride, from 4-10 vol. per cent of a material selected from the group consisting of benzene, toluene and xylene, and from 0.075 to 1 gram per 100 cc.

of solution of a synthetic rubber selected from the group consisting of polymers of chloroprene, copolymers of butadiene and styrene, and copolymers of chloroprene and isoprene.

3. Process for transparentizing paper which comprises applying a solution consisting of from 10-35 vol. per cent mineral oil, from 55-80 vol. per cent carbon tetrachloride, from 4-10 vol. per cent of a material selected from the group consisting of benzene, toluene and xylene, and from 0.075 to 1 gram per 100 cc. of solution of a synthetic rubber selected from the group con-

sisting of polymers of chloroprene, copolymers of butadiene and styrene, and copolymers of chloroprene and isoprene to said paper.

5 References Cited in the file of this patent

UNITED STATES PATENTS

| Number    | Name      | Date          |
|-----------|-----------|---------------|
| 1,233,334 | Fehringer | July 17, 1917 |
| 2,400,612 | Sprague   | May 21, 1946  |
| 2,495,135 | Rodman    | Jan. 17, 1950 |